

Sept. 20, 1966

A. WÖGERBAUER

3,273,976

SHEET STEEL AND SECTIONS, TUBES AND COMPOSITE CONSTRUCTIONS  
MANUFACTURED THEREFROM

Filed March 16, 1964

6 Sheets-Sheet 1

FIG. 1



FIG. 2



FIG. 3



INVENTOR  
ALFRED WÖGERBAUER  
BY

*Brownbaugh, Free, Grawit & Donohue*  
HIS ATTORNEYS

Sept. 20, 1966

A. WÖGERBAUER

3,273,976

SHEET STEEL AND SECTIONS, TUBES AND COMPOSITE CONSTRUCTIONS  
MANUFACTURED THEREFROM

Filed March 16, 1964

6 Sheets-Sheet 2



FIG. 4



FIG. 5



FIG. 6



FIG. 7



FIG. 8

INVENTOR  
ALFRED WÖGERBAUER  
BY

*Brueckl, Frey, Janner & Dornbusch*

HIS ATTORNEYS

Sept. 20, 1966

A. WÖGERBAUER

3,273,976

SHEET STEEL AND SECTIONS, TUBES AND COMPOSITE CONSTRUCTIONS  
MANUFACTURED THEREFROM

Filed March 16, 1964

6 Sheets-Sheet 3

FIG. 9



FIG. 10



FIG. 11



INVENTOR  
ALFRED WÖGERBAUER  
BY

*Brennhaug, Free, Grav, Toloshaue*

HIS ATTORNEYS

Sept. 20, 1966

A. WÖGERBAUER

3,273,976

SHEET STEEL AND SECTIONS, TUBES AND COMPOSITE CONSTRUCTIONS  
MANUFACTURED THEREFROM

Filed March 16, 1964

6 Sheets-Sheet 4

FIG. 12



FIG. 13



FIG. 14

FIG. 15



FIG. 16



FIG. 17

INVENTOR  
ALFRED WÖGERBAUER  
BY

Brennagh, Free, Jones & Dorothy

HIS ATTORNEYS

Sept. 20, 1966

A. WÖGERBAUER

3,273,976

SHEET STEEL AND SECTIONS, TUBES AND COMPOSITE CONSTRUCTIONS  
MANUFACTURED THEREFROM

Filed March 16, 1964

6 Sheets-Sheet 5

FIG. 18



FIG. 19



FIG. 20



INVENTOR  
ALFRED WÖGERBAUER  
BY

*Brennagh Free, Deans & Donohue*

HIS ATTORNEYS

Sept. 20, 1966

A. WÖGERBAUER

3,273,976

SHEET STEEL AND SECTIONS, TUBES AND COMPOSITE CONSTRUCTIONS  
MANUFACTURED THEREFROM

Filed March 16, 1964

6 Sheets-Sheet 6



FIG. 21



FIG. 22

INVENTOR  
ALFRED WÖGERBAUER  
BY

*Brunnholz, Frei, Jäger & Dondorf*

HIS ATTORNEYS

# United States Patent Office

3,273,976

Patented Sept. 20, 1966

1

3,273,976

## SHEET STEEL AND SECTIONS, TUBES AND COMPOSITE CONSTRUCTIONS MANUFACTURED THEREFROM

Alfred Wogerbauer, Linz, Austria, assignor to Vereinigte Österreichische Eisen- und Stahlwerke Aktiengesellschaft, Linz, Austria, a company of Austria

Filed Mar. 16, 1964, Ser. No. 351,932

Claims priority, application Austria, Mar. 19, 1963,

A 2,166/63

6 Claims. (Cl. 29—180)

This invention relates to steel sheets and sections, tubes and composite constructions manufactured therefrom, having a yield point of more than 50 kg./sq.mm., a tensile strength of more than 55 kg./sq.mm., and an elongation of at least 8%.

For steel sheet and structural members having the mentioned parameters only steels of special grades, such as St 60 or St 70, which are classified as low alloy steels, and heat treatable steels, which have a higher content of alloy elements, such as manganese and vanadium, have hitherto been used. Steels having the mentioned characteristics, i.e. the low alloy structural steels and the higher alloy heat treatable steels, had to have a carbon content of considerably more than 0.30%, in order to achieve the required strength values. Steels having such high carbon content, however, can no longer be welded, or they require a special melting treatment, which materially increases the manufacturing costs and, consequently, the price of these steels.

It has been known that by cold working steel sheet or strips the strength values of these materials can be increased. As cold working measures it has been proposed to stretch, roll or draw the strip. During cold rolling the thickness or gauge of the sheets is reduced in several passes, this requiring voluminous and expensive installations. Also the hardening by cold stretching is a time consuming and uneconomical process which causes an undesirable loss of material due to the requirement of gripping the sheets. Drawing the sheets on drawing benches has not proved satisfactory either. This process was limited to comparatively narrow strips, a lot of waste material resulting for the same reasons as in stretching; furthermore lubrication is an unsolved problem in drawing processes.

It is further known to provide steel sheets with ornamental patterns by coining or stamping. A stamped sheet is, for instance, the so-called hammered sheet. By this process an increase of the strength values is obtained as a secondary effect. Primarily, however, the object of the known process is to obtain decorative effects.

As a further measure of strain-hardening sheet steel by cold working it has been proposed to impart to a hot rolled strip a ridge-and-groove profile by drawing or rolling, then flattening the ridge-and-groove profile and finally shaping the steel sheet treated in this way into sections. Flattening the ridge-and-groove profile causes, however, a change of width of the strips, depending on the groove depth chosen for profiling.

Finally, strain hardened steel sheet having lasting ridge-and-groove profiles or a buckled surface are known, which have been used for special construction purposes.

Up to now, it has not been possible, however, to achieve and guarantee to the buyers reproducible results. Due to the cold working the material frequently became so brittle that it could no longer be processed, as the yield point was highly increased, whereas the elongation at break was reduced to nil. Such a material is no longer useful for the manufacture of sections, tubes and composite constructions.

2

It is an object of this invention to avoid the disadvantages and difficulties described. The invention is based on the recognition that the degree of deformation of a cold working treatment used for strain hardening has to range between specific limits, in order to ensure a reproducibility of the results, particularly of the pair of values: yield point—elongation, which is of practical importance.

Accordingly, the invention provides a sheet steel and sections, tubes and composite constructions manufactured therefrom, respectively, having a yield point of more than 50 kg./sq.mm., a tensile strength of more than 55 kg./sq.mm., and an elongation of at least 8% which are characterized in that the work pieces consist of steel having a carbon content of less than 0.30%, and are provided with a ridge-and-groove profile in which the inner radius of curvature of the grooves is smaller than three times the sheet or wall thickness and the ratio of depth to pitch of the ridge-and-groove profile amounts to 1:15 to 1:3.

In particular, it is proposed for the composition of the material that the carbon content is 0.15 to 0.19%, the silicon content 0.06 to 0.15%, the manganese content 0.30 to 0.45%, the phosphorus content less than 0.09%, preferably not more than 0.03%, and the sulphur content less than 0.06%, preferably not more than 0.04%.

The strength values obtained by the cold working are in a certain relation also with the sheet thickness. Under the mentioned conditions the sheet thickness should be 1 to 6 mm., preferably 1.5 to 4 mm.

In order to ensure the weldability of such work pieces, it is provided according to a further proposal of the invention that a steel strip provided according to the invention with a ridge-and-groove profile remains non profiled in narrow marginal zones, these zones serving for the welding in the subsequent manufacture of tubes, composite constructions, etc.

The effect of the ridge-and-groove profiling according to the invention is essentially due to the fact that the profiled work piece is alternately bent and stretched perpendicularly to the direction of the ridges and grooves, the bent zones corresponding in the proportion of half the pitch to the grooves and the stretched zones being interposed.

The invention is explained in more detail in the drawings. FIGS. 1, 2 and 3 are sectional views of ridge-and-groove profiled strips as viewed perpendicularly to the direction of the grooves. FIGS. 4 to 8 diagrammatically illustrate in like representation the manufacture of such strips. In FIGS. 9, 10 and 11 perspective views of sheets having different groove directions are shown. FIGS. 12 to 17 show, partly in sectional view and partly in top view, composite constructions made of strips provided according to the invention with a ridge-and-groove profile. FIGS. 18 to 20 represent other composite constructions in perspective view, and FIGS. 21 and 22 illustrate a process and an apparatus for manufacturing compound sheets.

In FIGS. 1 to 3, letter *d* denotes the sheet thickness, *r* the inner radius of curvature of the grooves, *t* the depth of the grooves and *a* the pitch of the ridge-and-groove profile, varying ratios of *r:d* and *t:a* being represented in the three figures.

In FIGS. 4 to 8 the individual steps of the manufacture of such ridge-and-groove profiled sheets and the formation of edged and stretched zones in the profiled sheet are illustrated. The originally unworked sheet 1 is passed into the roll gap between upper roll 2 and lower roll 3 and initially engaged by the rolls in such manner that the ridge-and-groove profile provided on the working surface of the rolls contacts the sheet with its ridges. In this

position the roll gap is designated by  $A_0$  (FIG. 4). When the roll gap is reduced (roll gap  $A_1$  in FIG. 5 and roll gap  $A_2$  in FIG. 6), the sheet 1 is continuously bent around the crests of the ridges, any peripheral recession from the edges of the strip being eliminated. The layer 4 originally disposed in the center of the sheet increases in length between two adjacent bends, so that the sheet is edged on the inside of the bending zones and is stretched on the outsides of the bending zones as well as in the interposed non-bent zones in the proportion of half the pitch. In this way the sheet is strain-hardened across its entire cross-section. Upon decreasing the roll gap the yield point and the tensile strength are increased, while the elongation decreases. The difference between the original roll gap  $A_0$  and a reduced roll gap  $A_1$  or  $A_2$  amounts to the groove depth applied to the sheet (indentation), which in FIGS. 1 and 2 is designated by  $t$ . The groove depth  $t$  plus the initial sheet thickness amounts to the nominal thickness  $s$  of the strain hardened sheet (FIG. 6). If the roll gap is reduced by further screwing down of the upper roll to such an extent that it is completely filled with the strain hardened sheet ( $A_4$  in FIG. 7), the alternating bending and transverse stretching is finished. Upon a further reduction of the roll gap, e.g., to  $A_5$  in FIG. 7, a breakdown rolling is superimposed to the finished phase of strain hardening. This results in a further increase of the strength values and enables a sizing of the sheet thickness, whereby it is possible to avoid deviations from the desired thickness which usually occur in hot rolled sheets and to achieve the same accuracy of the thickness dimensions as in cold rolled strips.

In FIG. 8 an extreme case is illustrated, wherein a sheet is strain hardened solely by alternating bending. The bent zones immediately adjoin to each other, without having zones of pure stretch drawing interposed therebetween, which may be accomplished by a suitable choice of the variable process conditions (adjustment of the roll gap relative to the sheet thickness).

In the following examples, the yield point, tensile stress and elongation values obtained in steel sheets of grades St 37, St 42 and St 44 are given. In several tests the dimensions of inner radius  $r$  of curvature, sheet thickness  $d$ , groove depth  $t$  and pitch  $a$  were varied; the exact chemical composition of the material is likewise given.

Example 1.—Strip No. 948,569, chemical composition: 0.01% C, 0.11% Si, 0.29% Mn, 0.009% P, 0.020% S (St 42).

| Test No. | $a$ | $r$  | $t$  | $d \rightarrow s$ | $\sigma_s$ | $\sigma_z$ | $\delta$ |
|----------|-----|------|------|-------------------|------------|------------|----------|
| 1a       | 5   | 1.25 | 0.00 | 1.81              | 41.0       | 45.1       | 27.2     |
| 2        | 5   | 1.25 | 0.40 | 2.21              | 53.9       | 55.0       | 8.2      |
| 3        | 5   | 1.25 | 0.46 | 2.27              | 53.9       | 56.2       | 10.7     |
| 4        | 5   | 1.25 | 0.55 | 2.36              | 53.8       | 56.5       | 9.5      |
| 5        | 5   | 1.25 | 0.61 | 2.42              | 54.6       | 57.2       | 8.0      |
| 6        | 5   | 1.25 | 0.65 | 2.46              | 55.6       | 58.2       | 8.5      |

a Initial value (non-hardened sheet).

Example 2.—Strip No. 948,567, chemical composition: 0.12% C, 0.09% Si, 0.35% Mn, 0.011% P, 0.025% S (St 42).

| Test No. | $a$ | $r$  | $t$  | $d \rightarrow s$ | $\sigma_s$ | $\sigma_z$ | $\delta$ |
|----------|-----|------|------|-------------------|------------|------------|----------|
| 1a       | 5   | 1.25 | 0.00 | 1.84              | 33.6       | 44.5       | 30.5     |
| 2        | 5   | 1.25 | 0.50 | 2.34              | 55.5       | 57.2       | 8.2      |
| 3        | 5   | 1.25 | 0.56 | 2.40              | 55.0       | 57.3       | 8.2      |
| 4        | 5   | 1.25 | 0.61 | 2.45              | 56.0       | 57.6       | 7.9      |

a Initial value (non-hardened sheet).

Example 3.—Strip No. 948,572, chemical composition: 0.09% C, 0.13% Si, 0.45% Mn, 0.012% P, 0.026% S, 0.004% N (St 42).

| Test No. | $a$ | $r$  | $t$  | $d \rightarrow s$ | $\sigma_s$ | $\sigma_z$ | $\delta$ |
|----------|-----|------|------|-------------------|------------|------------|----------|
| 1a       | 5   | 1.25 | 0.00 | 1.78              | 32.4       | 43.4       | 30.7     |
| 2        | 5   | 1.25 | 0.42 | 2.20              | 54.4       | 55.1       | 8.6      |
| 3        | 5   | 1.25 | 0.52 | 2.30              | 54.0       | 55.0       | 8.0      |

a Initial value (non-hardened sheet).

Example 4.—Strip No. 948,568, chemical composition as in Example 2.

| Test No. | $a$ | $r$  | $t$  | $d \rightarrow s$ | $\sigma_s$ | $\sigma_z$ | $\delta$ |
|----------|-----|------|------|-------------------|------------|------------|----------|
| 1a       | 5   | 1.25 | 0.00 | 1.86              | 33.7       | 44.8       | 33.5     |
| 2        | 5   | 1.25 | 0.40 | 2.26              | 52.4       | 55.6       | 8.5      |
| 3        | 5   | 1.25 | 0.45 | 2.31              | 53.1       | 55.0       | 11.0     |
| 4        | 5   | 1.25 | 0.50 | 2.36              | 56.3       | 57.2       | 9.2      |

a Initial value (non-hardened sheet).

Example 5.—Chemical composition: 0.16% C, 0.09% Si, 0.32% Mn, 0.09% P and 0.025% S (St 42).

| Test No.          | $a$ | $r$ | $t$ | $d$ | $\sigma_s$  | $\sigma_z$  | $\delta$ |
|-------------------|-----|-----|-----|-----|-------------|-------------|----------|
| Starting material | mm. | mm. | mm. | mm. | kg./sq. mm. | kg./sq. mm. | percent  |
| Strain hardened   | 4   | 1.6 | 0.6 | 1.5 | 57.6        | 58.6        | 8.5      |

Example 6.—Chemical composition as in Example 5.

| Test No.          | $a$ | $r$ | $t$ | $d$ | $\sigma_s$  | $\sigma_z$  | $\delta$ |
|-------------------|-----|-----|-----|-----|-------------|-------------|----------|
| Starting material | mm. | mm. | mm. | mm. | kg./sq. mm. | kg./sq. mm. | percent  |
| Strain hardened   | 4   | 1.6 | 0.4 | 1.5 | 53.9        | 57.4        | 9.9      |

Example 7.—Chemical composition as in Example 5.

| Test No.          | $a$ | $r$ | $t$ | $d$ | $\sigma_s$  | $\sigma_z$  | $\delta$ |
|-------------------|-----|-----|-----|-----|-------------|-------------|----------|
| Starting material | mm. | mm. | mm. | mm. | kg./sq. mm. | kg./sq. mm. | percent  |
| Strain hardened   | 10  | 2.5 | 1.4 | 1.5 | 55.4        | 62.5        | 12.3     |

Example 8.—Chemical composition as in Example 5.

| Test No.          | $a$ | $r$  | $t$ | $d$ | $\sigma_s$  | $\sigma_z$  | $\delta$ |
|-------------------|-----|------|-----|-----|-------------|-------------|----------|
| Starting material | mm. | mm.  | mm. | mm. | kg./sq. mm. | kg./sq. mm. | percent  |
| Strain hardened   | 10  | 3.15 | 2.4 | 1.5 | 63.5        | 64.7        | 8.0      |

Example 9.—Chemical composition: 0.10% C, 0.11% Si, 0.29% Mn, 0.009% P and 0.020% S (St 42).

| Test No. | $a$ | $r$  | $t$ | $d$ | $\sigma_s$ | $\sigma_z$ | $\delta$ |
|----------|-----|------|-----|-----|------------|------------|----------|
| 1        | 4   | 1.6  | 0.5 | 1.7 | 53.8       | 55.0       | 9.6      |
| 2        | 5   | 1.25 | 0.6 | 1.6 | 54.3       | 59.0       | 8.3      |
| 3        | 6   | 2.25 | 1.1 | 1.6 | 58.4       | 61.6       | 9.1      |
| 4        | 6   | 2.25 | 1.3 | 1.6 | 59.3       | 60.6       | 8.2      |
| 5        | 8   | 2.75 | 1.3 | 1.6 | 56.5       | 58.6       | 8.0      |
| 6        | 8   | 2.75 | 1.5 | 1.6 | 58.1       | 59.6       | 8.8      |
| 7        | 10  | 2.5  | 2.2 | 1.7 | 59.6       | 61.2       | 10.2     |
| 8        | 10  | 2.5  | 2.3 | 1.7 | 59.9       | 61.3       | 8.9      |

The results of further tests using sheet steel of grade St 44 are evident from the following table:

Chemical composition: 0.17% C, 0.25% Si, 0.68% Mn, 0.025% P, 0.028% S, 0.0055% N (St 44).

|                   | <i>a</i> | <i>r</i> | <i>t</i> | <i>d</i> | $\sigma_s$  | $\sigma_z$  | $\delta$ |
|-------------------|----------|----------|----------|----------|-------------|-------------|----------|
|                   | mm.      | mm.      | mm.      | mm.      | kg./sq. mm. | kg./sq. mm. | percent  |
| Starting material |          |          |          | 1.87     | 35.5        | 51.8        | 28.5     |
| Strain hardened   | 4        | 1        | 0.12     | 1.99     | 50.7        | 55.0        | 20.7     |
| Starting material |          |          |          | 1.85     | 38.0        | 52.4        | 26.3     |
| Strain hardened   | 4        | 1        | 0.16     | 2.01     | 51.6        | 55.8        | 19.4     |
|                   | 4        | 1        | 0.16     | 2.01     | 52.2        | 55.6        | 21.2     |
|                   | 4        | 1        | 0.16     | 2.01     | 51.8        | 55.2        | 19.4     |
|                   | 4        | 1        | 0.16     | 2.01     | 51.1        | 55.1        | 20.5     |
| Starting material |          |          |          | 1.85     | 37.6        | 52.6        | 25.4     |
| Strain hardened   | 4        | 1        | 0.2      | 2.05     | 55.0        | 56.8        | 15.1     |
|                   | 4        | 1        | 0.2      | 2.05     | 55.3        | 57.0        | 14.5     |
|                   | 4        | 1        | 0.2      | 2.05     | 55.9        | 57.4        | 12.0     |
|                   | 4        | 1        | 0.2      | 2.05     | 54.6        | 56.8        | 16.5     |
| Starting material |          |          |          | 1.85     | 37.0        | 51.8        | 27.6     |
| Strain hardened   | 4        | 1        | 0.24     | 2.09     | 58.4        | 60.2        | 9.5      |
|                   | 4        | 1        | 0.24     | 2.09     | 58.4        | 60.4        | 9.9      |
|                   | 4        | 1        | 0.24     | 2.09     | 57.0        | 58.7        | 12.4     |
|                   | 4        | 1        | 0.24     | 2.09     | 58.6        | 60.1        | 10.1     |
| Starting material |          |          |          | 1.83     | 36.6        | 51.4        | 29.1     |
| Strain hardened   | 4        | 2        | 0.2      | 2.03     | 53.0        | 55.5        | 18.4     |
|                   | 4        | 2        | 0.2      | 2.03     | 53.6        | 55.8        | 19.5     |
| Starting material |          |          |          | 1.85     | 36.2        | 51.9        | 29.9     |
| Strain hardened   | 4        | 2        | 0.3      | 2.15     | 56.8        | 58.8        | 15.0     |
|                   | 4        | 2        | 0.3      | 2.15     | 55.7        | 58.6        | 15.0     |
| Starting material |          |          |          | 1.85     | 36.8        | 51.6        | 30.1     |
| Strain hardened   | 4        | 2        | 0.4      | 2.25     | 58.7        | 60.6        | 12.1     |
| Starting material |          |          |          | 1.85     | 35.6        | 51.4        | 28.5     |
| Strain hardened   | 5        | 1.6      | 0.3      | 2.15     | 54.2        | 56.3        | 15.5     |
|                   | 5        | 1.6      | 0.3      | 2.15     | 54.3        | 56.3        | 17.9     |
| Starting material |          |          |          | 1.85     | 37.2        | 52.0        | 27.6     |
| Strain hardened   | 5        | 1.6      | 0.4      | 2.25     | 57.4        | 59.3        | 8.8      |
|                   | 5        | 1.6      | 0.4      | 2.25     | 57.9        | 59.2        | 11.7     |

In FIG. 9 a strip sheet is illustrated which comprises three zones having ridge-and-groove profiles running in crosswise directions. The lateral zones 6 and 7 are longitudinally grooved, and the interposed middle zone 8 is transversely grooved. The marginal zones 5 are nonprofiled and nonhardened so that they are easily weldable. Sheets of this type are particularly suitable for the manufacture of heat exchangers.

In FIG. 10 a strip sheet is shown, which comprises two nonprofiled (nonhardened) marginal zones 9 and 10 and an interposed middle zone 11. The middle zone 11 has crossing diagonal grooves 12, 12'. A similar design is shown in FIG. 11. There, the middle zone 11 is again provided between two nonhardened marginal zones 9 and 10 of a sheet strip and has superimposed ridge-and-groove profiles 13, 13'.

FIGS. 12 to 14 illustrate in two sectional views and in a plan view a compound sheet consisting of a longitudinally grooved upper sheet 15 and a transversely grooved lower sheet 16. These sheets are connected to each other at the points of intersection 17 of the longitudinal ridges with the transverse ridges by welding, preferably resistance welding.

In FIGS. 15 and 16 again a compound sheet is shown which consists of three single sheets strain hardened by a ridge-and-groove profile. Between a longitudinally grooved upper sheet 18 and a likewise longitudinally grooved lower sheet 19 a transversely grooved intermediate sheet 20 is arranged. The three sheets are connected with each other at the points of intersection of the ridges by welding.

FIG. 17 shows a composite body of the hollow panel type. It consists of a longitudinally grooved upper sheet 21, a likewise longitudinally grooved lower sheet 22 and a zigzag-shaped middle part 23 serving as a spacer and forming a strutting. The middle part 23 may also be made of a transversely grooved sheet so that at the junctions of the middle part with the sheets 21 and 22 longitudinal and transverse ridges again intersect and can be connected in a simple manner by resistance welding.

FIGS. 18, 19 and 20 illustrate other structural panels formed of sandwich boards of the type shown in FIGS. 12 and 13. In FIG. 18 a trapezoidally bent middle part 26 is arranged between an upper compound sheet 24 and a lower compound sheet 25, the middle part consisting of a single, longitudinally grooved sheet. Similarly, in FIG. 19 a middle part 29 of transversely grooved sheet is welded in between the two compound sheets 27 and 28. FIG. 20 shows a structural panel, in which not only the outer sheets 30 and 31, but also the middle part 32 consist of a compound sheet of the type illustrated in FIGS. 12 and 13.

In FIG. 21 an apparatus for the continuous manufacture of compound sheets, e.g. of the type shown in FIGS. 12 and 13, is illustrated. The apparatus comprises reels for unwinding coiled hot rolled strips, devices for applying a ridge-and-groove profile viz. selectively a longitudinal or a transverse ridge-and-groove profile, a welding equipment for connecting the ridge-and-groove profiled single sheets, and a device for winding up or for shearing to length the composite constructions. The strip 54 is reeled off coil 55, and simultaneously strip 56 is reeled off coil 57. The strip 54 comes via the reversing roller 58 to the transverse-grooving rolls 59 and 60, in the roll gap of which it is imparted a transverse ridge-and-groove profile and strain-hardened. Upon strain-hardening, the strip 54 is taken off via the reversing rollers 61 and 62. Simultaneously the strip 56 is fed via the reversing roller 63 into the roll gap of a two-high stand comprising rolls 64 and 65. The longitudinal-grooving rolls 64 and 65 impart to the strip a ridge-and-groove profile in the longitudinal direction. Arranged behind the two-high there may be a four-high stand comprising the backing-up rolls 66 and 67 and the breaking-down rolls 68 and 69. The longitudinally grooved sheet 70 now is passed straight on to the welding equipment, where it meets with the first strip, here designated by numeral 71, which is fed via the reversing roller 72. The speed of the two strips must be synchronized, which may be accomplished by means of known type. Such a synchronizing means is indicated in FIG. 21 by the roll 72 being displaceable from the position drawn in fully inked lines to the position drawn in dash lines. The shortening and lengthening, respectively, of the loop formed by the transversely grooved strip 71 which is due to the movability of roll 72, may be utilized for synchronizing.

The welding equipment comprises the current supply roller 73 and the current supply roller 74. To these two electrode rollers welding current is supplied from the transformer 75 via the sliding contacts 76 and 77. The electrode rollers extend over the entire width of the strips 70 and 71, which are continuously passed through between the electrode rollers in superposed position. Owing to the power concentration at the points of intersection of the longitudinal ridges with the transverse ridges of the two superposed sheets 70 and 71, transverse rows of intersections are successively welded together. For welding, alternating current or, preferably, direct current may be used. The welded compound sheet 78 may be cut behind the welding machine into sheets of desired length by means of blades 79 and 80.

In FIG. 22 the gap between the electrode rollers is illustrated on an enlarged scale. Numerals 81 and 82 denote the course of the welding current, which is concentrated at the crossing point 83 and there welds together sheets 70 and 71.

Composite constructions according to the present invention may be used with advantage in building practice for walls, ceilings, doors, gates, as clothing or the like. A preferred field of application further lies in car building. In addition to the advantages of the invention already mentioned which are manifested by an increase of the strength properties and a simultaneous maintenance of an elongation sufficient for shaping operations, it is to be remarked that the building safety of buildings made with structural elements according to the present invention is increased and a favorable architectural effect is achieved. Moreover, the costs, as compared with those of known structural elements which had to be made of considerably more expensive materials, are materially lower.

What I claim is:

1. Strain hardened sheet steel having a yield point of more than 50 kg./mm., a tensile strength of more than 55 kg./sq. mm., and an elongation of at least 8%, the sheet steel being made of steel having a carbon content of less than 0.30% and being provided with a ridge-and-groove profile in which the inner radius of curvature of the grooves is smaller than three times the sheet thickness and the ratio of depth to pitch of the ridge-and-groove profile amounts to 1:15 to 1:3.

2. Sections, tubes and composite constructions made of sheet steel as set forth in claim 1.

3. Strain hardened sheet steel having a yield point of more than 50 kg./sq. mm., a tensile strength of more than 55 kg./sq. mm., and an elongation of at least 8%, the sheet steel being made of steel having a carbon content of 0.15 to 0.19%, a silicon content of 0.06 to 0.15%, a manganese content of 0.30 to 0.45%, a phosphorus content of less than 0.09%, and a sulphur content of less than 0.06% and being provided with a ridge-and-groove profile in which the inner radius of curvature of the grooves is smaller than three times the sheet thickness and the ratio of depth to pitch of the ridge-and-groove profile amounts to 1:15 to 1:3.

4. The sheet steel as set forth in claim 3 in which the

phosphorus content is not more than 0.03% and the sulphur content is not more than 0.04%.

5. Sheet steel in the form of strain hardened strip having a yield point of more than 50 kg./sq. mm., a tensile strength of more than 55 kg./sq. mm., and an elongation of at least 8%, the sheet steel being made of steel having a carbon content of 0.15 to 0.19%, a silicon content of 0.06 to 0.15%, a manganese content of 0.30 to 0.45%, a phosphorus content of less than 0.09%, and a sulphur content of less than 0.06%, having a sheet thickness of 1 to 6 mm, and being provided with a ridge-and-groove profile in the longitudinal direction of the strip leaving free narrow marginal zones, the inner radius of curvature of the grooves being smaller than three times the sheet thickness and the ratio of depth to pitch of said ridge-and-groove profile amounting to 1:15 to 1:3.

6. Strain hardened sheet steel having a yield point of more than 50 kg./sq. mm., a tensile strength of more than 55 kg./sq. mm., and an elongation of at least 8%, the sheet steel being made of steel having a carbon content of less than 0.30% and being provided with a ridge-and-groove profile in which the inner radius of curvature of the grooves is smaller than three times the sheet thickness and the ratio of depth to pitch of the ridge-and-groove profile amounts to 1:15 to 1:3, said sheet steel comprising perpendicularly to the direction of the grooves, alternating bent and stretched zones in relation to the pitch of the grooves, the bent zones corresponding in the proportion of half the pitch to the grooves and the stretched zones being interposed.

#### References Cited by the Examiner

##### UNITED STATES PATENTS

|           |         |           |       |        |
|-----------|---------|-----------|-------|--------|
| 1,868,302 | 7/1932  | Auger     | ----- | 29—180 |
| 1,982,243 | 11/1934 | Black     | ----- | 29—180 |
| 2,089,242 | 8/1937  | Whitesell | ----- | 29—180 |
| 2,160,677 | 5/1939  | Romanoff  | ----- | 29—180 |

DAVID L. RECK, Primary Examiner.

HYLAND BIZOT, R. O. DEAN, Assistant Examiners.